

Aug. 11, 1953

G. H. SWART

2,648,084

REINFORCED WIRE BRUSH

Filed May 4, 1949



INVENTOR

Gilbert H. Swart

BY

Evans & McCoy  
ATTORNEYS

Fig. 4

## UNITED STATES PATENT OFFICE

2,648,084

## REINFORCED WIRE BRUSH

Gilbert H. Swart, Akron, Ohio, assignor to The  
General Tire and Rubber Company, Akron,  
Ohio, a corporation of Ohio

Application May 4, 1949, Serial No. 91,280

5 Claims. (Cl. 15—198)

1

This invention relates to improvements in metal brushes such as are used for polishing and cleaning of metal and other articles. It particularly relates to wire brushes having improved operating characteristics and to a method of preparing such brushes.

Enormous quantities of wire brushes are utilized for the cleaning and polishing of metal articles, castings and the like. These brushes have much shorter life than would be expected because of normal wear on the cutting or cleaning edges of the bristles. They are frequently subjected to moisture which causes rusting and deterioration of the wires. When they are subjected to extra hard usage or to considerable pressure in the polishing or cleaning operation, the flexing of the wires frequently becomes so severe that a great deal of filament breakage may occur. It is for these reasons it has been thought that an improvement might result if the bristles were completely embedded in a rubber compound. However, it is exceedingly difficult, if not impossible, to embed bristles in a rubber compound for the reason that in any molding operation the flow of rubber tends to greatly distort the bristle pattern, with the result that the brush may have an uneven cutting path. Furthermore, rubber compounds usually contain sulfur that reacts with iron wire and they have very substantial abrasion resistance, which is frequently substantially greater than the abrasion resistance of steel. With such a high abrasion resistance the bristles can wear off below the surface of the rubber and the desirable characteristics of a wire brush are not obtained. This even though the bristles may be protected from the elements and give sufficient rigidity so that their life is greatly enhanced.

It is an object of the present invention to provide a wire brush in which the wire bristles are substantially completely embedded and are reinforced against flexure by a composition which has substantial strength, which protects them from the elements and from most corrosive fluids, but which has a sufficiently lower abrasion resistance than does metal so that it does not noticeably interfere with the operations for which the ends of wire bristles are especially suited.

It is another object of the present invention to provide a wire brush having the bristles reinforced and protected from the elements by a composition which is not susceptible to deterioration by grease and other liquids with which such brushes may come in contact, and which while

2

having relatively high strength has sufficiently lower abrasion resistance than metal to wear sufficiently to expose the cutting edges of the wire so that the wire bristles take substantially all of the abrasion in the operation of the brush.

Other objects will be apparent from the following description of the invention as illustrated in the accompanying drawing, in which:

Figure 1 is a plan view of a mold containing a wire brush embodying the present invention and suitable for the final step in the manufacture of one form of wire brush (rotary) embodying the present invention;

Fig. 2 is a sectional view on the line 2—2 of Fig. 1;

Fig. 3 is a plan view of a portion of a brush embodying the present invention; and

Fig. 4 is a sectional view on the line 4—4 of Fig. 2.

I have found that the above objects are accomplished by immersing the entire bristle portion of the conventional wire brush in a fluid comprising a polymerizable or copolymerizable polyester or condensation polymer and capable of setting or changing by molecular growth from the liquid to the solid state and then causing the solidification while the bristles are substantially completely embedded therein. The wire brush body is preferably incorporated in a suitable mold and a fluid polyester mixture or condensation polymer of the type capable of solidification by molecular growth may be added to the mold in sufficient volume to completely envelop the bristle portions of the brush. It is polymerized or solidified in contact with the bristles to embed them in a solid matrix.

I have found that the solids polymerized from a mixture comprising an unsaturated polyester and a copolymerizable monoolefinic compound, when solidified in situ throughout the bristle portions of the wire brushes, greatly improve the operation of such brushes. These solidified condensation polymers are exceptional in that they have almost no abrasion resistance and yet have relatively high strength and resistance to deterioration against chemical attack in various fluids. They need contain no sulfur or chemicals that react with metal and because of their low abrasion resistance they wear down much more readily than do the wire bristles, with the result that the ends of the wire are exposed and the operation of the wire brushes is not adversely interfered with. They enhance the cutting and cleaning operations of the wire brushes for the

reason that they greatly stiffen the wire bristles and prevent their deterioration by flexing.

The condensation polymers which are rubbery are particularly effective and are preferred. The copolymers of linear polyesters containing unsaturated linkages with mono-olefinic compounds, such as styrene, methyl methacrylate, methyl acrylate and acrylonitrile, are exceptional. These linear polyesters usually comprise a polyhydric alcohol, preferably a dihydric alcohol such as ethylene glycol, di- and tri-ethylene glycols, etc., and a mixture of any one or more saturated and any one or more unsaturated dibasic acids.

The saturated dibasic acid is preferably any dicarboxylic acid of a sufficient number of carbon atoms to prevent formation with the dihydric alcohols of a five, six or seven-numbered ring, and usually has at least four carbon atoms. Examples of such acids are adipic acid, sebacic acid, phthalic acid, terphthalic acid, etc., although any dicarboxylic acid may be used providing the alcohols are chosen to prevent ring formation. The saturated acids generally comprise a major proportion of the acidic material. The unsaturated dibasic acids, of which maleic and fumaric acids are examples, comprise generally a minor portion of the composition and are present merely to provide crosslinking points for polymerization with a suitable mono-olefinic compound, such as styrene, etc. The amount of unsaturation has a direct bearing on the shrinkage during the casting process, hence it is desirable to have the unsaturated acid as low as compatibility with styrene or mono-olefinic component permits. The mono-olefinic component which copolymerizes with the polyesters of the preferred type to crosslink the fluid polyester and assist in its conversion to the solid state may be any polymerizable mono-olefinic compound or any mono-olefinic compound copolymerizable with maleic anhydride. Examples of such are the acrylic and methacrylic esters and nitriles, styrenes, polymerizable nuclearly substituted styrenes, including all the chlorostyrenes, the corresponding alpha-alkylstyrenes, etc.

The polyester components are usually prepared by first condensing a polyhydric alcohol and a mixture of dibasic acids, or their anhydrides, to form a liquid-to-viscous polyester which is preferably largely of linear nature. This polyester is generally condensed by stirring the mixture of reactants while heated to boiling until the boiling point of the reactants becomes well over 200° C., where it is evident that most of the water formed by the condensation reaction is removed as soon as it is formed. The container in which the esterification reaction generally occurs is fitted with a suitable reflux condenser which operates at a sufficiently high temperature to condense only the organic constituents and to permit the escape of water vapor. The molecular weight of the polyester thus obtained is determined largely by the proportion of the reactants, the highest molecular weight being obtained with an exact balance of hydroxyl and carboxyl groups.

In place of part or even all of the polyhydric alcohols and polybasic acids, a hydroxy carboxylic acid having sufficient space between the carboxyl and hydroxyl groups to prevent formation of five, six or seven-numbered rings may be condensed alone, providing a small amount of unsaturated linkages is provided, either by mixture of a small amount of unsaturated acid with

dihydric alcohol or by the use of suitable unsaturated hydroxy aliphatic acids.

The hardness of the plastic composition may be determined by the relative proportion of mono-olefinic monomer that is mixed with the polyester and about equal proportions, by weight, or from 30 parts of polyester to 70 parts of styrene or mono-olefinic monomer, to 30 parts of styrene and 70 parts of polyester are quite satisfactory. The rubber properties are enhanced by increasing the amount of polyester, and the hardness is enhanced by increasing the proportion of styrene or mono-olefinic component. Generally a higher molar percentage of polyester than of styrene or mono-olefinic compound is preferred so that a rubbery type of material is had. The amount of shrinkage in the polyester is as aforesaid controlled largely by the amount of unsaturated dibasic acid in the polyester available for crosslinkage. About 5% to 5% is preferred, although the amount of unsaturated dibasic acid may be as much as 25% or even more of the polyester.

Referring particularly to the drawing, wherein like parts are designated by like numerals of reference throughout the several views, a brush 10, the improvement of which the present invention is concerned, comprises a handle or hub portion 1, which may have an opening 2 to receive a suitable shaft or handle, and suitable means, such as one or more locking rings 3 for retaining on the hub or handle 1 the wire bristles 4, which extend out from the hub or handle portion (and are generally radially therefrom in a rotary brush), all in accordance with conventional practice.

In accordance with the present invention, the spaces 5 between the bristles 4 are filled with a solid polymerization product or resin of the class above-described, which resin has been solidified in situ by molecular growth or by polymerization to substantially completely enclose all but the end portions of the various wire filaments in a unitary and solid mass.

In the manufacture of brushes embodying the present invention, the brush may be placed in a suitable mold 11 having a cavity adapted to receive the conventional wire brushes and being of such size that the bristles preferably bear against the wall of the cavity. The mold may have a lower portion 13 and a suitable cover 14, together with means such as lugs 15 and the nut 16 for fastening the cover 14 to the lower portion of the mold. A suitable gasket 17 may be applied on either side of the surface of the hub to form a seal and to prevent liquid from entering into the space 2 adapted to receive the shaft. Suitable means, such as the spaced collars 18 and the bolt 19, may be provided for applying pressure to seal the space between the external surface of the hub 1 and the parts of the mold.

After the conventional wire brush is incorporated in the mold and the mold sealed so that leakage is prevented into the shaft portion thereof, a fluid polymerizable composition as above-described and containing a suitable polymerization catalyst is poured through the opening or sprue hole 20 to completely surround and envelop all of the bristles. A vent 21 may be provided to enable escape of air from the mold. After the mold has been filled with fluid composition capable of being polymerized or solidified to the solid state, the fluid composition is converted by molecular growth to the solid state, either by allowing it to set at normal tempera-

tures until polymerization has occurred, or by heating it at slightly elevated temperatures.

The rate of polymerization is controlled by the catalyst incorporated in the composition. The higher the percentage of oxidation catalyst, such as organic soluble peroxide, for example benzoyl peroxide, tertiary butyl hydrogen peroxide, or any other suitable catalyst, the greater is the rate at which hardening occurs. The amount of catalyst preferably should not be greater than .5% of the weight of the polymerizable constituents and as little as .01% is quite effective, all as well-known to those skilled in this art.

In order to remove the solidified brush from the mold, the inner mold surface 25 should preferably be coated prior to incorporation of the brush therein with a suitable lubricating material, such for example as a cellulose acetate.

The following example illustrates the present invention:

A liquid polyester is prepared by heating 1.05 mols of diethylene glycol with .7 mol of adipic acid and .3 mol of maleic anhydride. While stirring in a vessel equipped with a reflux condenser, cooled by fluid maintained at a temperature of about 105° C. to permit escape of water vapor but to return higher boiling constituents to the reaction mixture, the mixture is heated sufficiently to maintain boiling conditions until the temperature reaches 225° C., whereupon the reaction mixture is allowed to cool. About 55 parts of the cooled reaction mixture is mixed with 45 parts by weight of styrene and .1 part of tertiary butyl hydroperoxide.

A conventional wire brush having bristles radially extending from the hub is incorporated in the cavity of the mold 11, which was coated throughout with a layer of cellulose acetate or any other suitable mold lubricant. In the mold the hub 1 bears against the gasket 17 and the external edges 26 of the bristles bear against the inner wall portion 25a. The fluid solidifiable composition is poured through the opening 20 until it rises within the vent 21. It is allowed to remain at 60° C. until it has completely solidified. The brush removed from the mold has exceptionally desirable properties. It has much more rapid cutting time and much superior life than any wire brushes of which I am aware.

As aforesaid, the condensation resinous materials, and particularly those of the polyester mono-olefinic type, such for example as the linear polyester of one or more dihydric alcohols and one or more dibasic acids, part of which may or may not be unsaturated, with a mono-olefinic compound such as styrene, give by far the most desirable properties. This is particularly true when the percentage of polyester is greater than the percentage of mono-olefinic compound. Mixtures of mono-olefinic compounds such as styrene, methyl acrylate, methyl methacrylate, may be used for one alone. Similarly, mixtures of polyhydric alcohols, such as ethylene glycol and/or glycerol with a polyethylene glycol may be used in place of one alone, and a single dicarboxylic acid or a mixture of several may be used, providing the mono-olefinic compound is compatible with the resultant liquid or viscous condensation product.

Although the invention may be employed in various ways, only preferred embodiments have been illustrated and described. Other embodi-

ments may be made within the invention as provided by the patent statutes.

What I claim is:

- 5 1. In a wire brush comprising a fastening portion and a plurality of wire bristles extending therefrom, the improvement which comprises a solid polymerization product of a mixture of a polyester of at least one compound selected from the group consisting of dibasic acids and dibasic acid anhydrides and at least one polyhydric alcohol and a mono-olefinic compound compatible and polymerizable therewith substantially completely surrounding and reinforcing the sides of said wire bristles and joining portions spaced from said fastening portion together.
  - 10 2. In a wire brush comprising a hub portion adapted to receive a shaft and a plurality of wire bristles extending in a general radial direction therefrom, the improvement which comprises a solid polymerization product of polyester of at least one compound selected from the group consisting of dibasic acids and dibasic acid anhydrides and at least one polyhydric alcohol and compatible mono-olefinic compound
  - 15 20 25 30 35 40 45 50 55 60 65 70 75 80 85 90 95
  3. In a wire brush comprising a hub portion adapted to receive a shaft and a plurality of wire bristles extending in a general radial direction therefrom, the improvement which comprises a solid polymerization product of a mixture of styrene and an unsaturated condensation product of at least one dibasic acid and at least one dihydric alcohol entirely surrounding said bristles and integrally bonding portions of said bristles radially spaced from said hub.
  4. In a wire brush comprising a hub portion adapted to receive a shaft and a plurality of wire bristles extending in a general radial direction therefrom, the improvement which comprises a solid polymerization product of a mixture of a monoolefinic compound polymerizable and compatible with an unsaturated condensation product of at least one dibasic acid, and at least one dihydric alcohol entirely surrounding said bristles and integrally bonding portions of said bristles radially spaced from said hub.
  5. In a wire brush comprising a hub portion adapted to receive a shaft and a plurality of wire bristles extending in a general radial direction therefrom, the improvement which comprises a solid polymerization product of a mixture of styrene and a fluid condensation product of a dihydric alcohol, an alpha-beta unsaturated dicarboxylic acid, and a saturated dicarboxylic acid entirely surrounding said bristles and integrally bonding portions of said bristles radially spaced from said hub.
  - 60 65 70 75 80 85 90 95
  6. GILBERT H. SWART.
- References Cited in the file of this patent
- UNITED STATES PATENTS
- | Number    | Name      | Date           |
|-----------|-----------|----------------|
| 1,308,330 | Brown     | July 1, 1919   |
| 1,764,662 | Tomlin    | June 17, 1930  |
| 2,130,948 | Carothers | Sept. 20, 1938 |
| 2,207,158 | Neville   | July 9, 1940   |
| 2,390,437 | Hayes     | Dec. 4, 1945   |
| 2,397,471 | Cox       | Apr. 2, 1946   |
| 2,413,219 | D'Alelio  | Dec. 24, 1946  |
| 2,426,315 | Marick    | Aug. 26, 1947  |